

# UNITED STATES PATENT OFFICE.

NICOLAS HENRI MARIE DEKKER, OF PARIS, FRANCE.

## ELECTROLYTE FOR USE IN ELECTROMETALLURGY.

1,113,546.

Specification of Letters Patent. Patented Oct. 13, 1914.

No Drawing.

Application filed August 17, 1912. Serial No. 715,593.

To all whom it may concern:

Be it known that I, NICOLAS HENRI MARIE DEKKER, subject of the Kingdom of the Netherlands, residing at 29 Rue de la Sourdére, Paris, France, have invented new and useful Improvements in or Relating to Electrolytes for Use in Electrometallurgy, of which the following is a specification.

In electrolytic operations secondary reactions are always found due to the decomposition of the water which in its turn is due to the presence of free acid in the bath, which acid favors the formation of hydrogen and oxygen which produce basic salts, 15 oxids, etc., which unfavorably affect the operation. Of all the usual metals, only one can be treated in a practical manner at the present time, namely copper which is generally produced in that way, but that production relates only to the refining of the "mattes," for it has not hitherto been possible to obtain copper by exhausting a complex electrolyte. The greatest difficulty at present met with in obtaining good electrolytic deposits, is therefore due to water dilutions without which no electrolysis have hitherto been undertaken and when it is desired to obtain by electrolysis a metal, by refining, the operation is always carried out 25 with baths obtained by dissolving in water a salt of the metal to be obtained to which are added one or more other salts of different metals generally of alkaline metals. In order to avoid that disadvantage, it has 30 been suggested to use hygroscopic salts, but without success, because that method always leads to secondary reactions due to the use of these salts or to hydrogen or oxygen or to both these gases produced by the decomposition of the water by the free acid. It has thus been found that hydrides, oxids or basic salts of zinc are formed during electrolysis of salts of zinc. In the same way, it has been found that basic salts or oxid of 35 iron are formed in the electrolysis of an iron salt.

In order to avoid the disadvantages due to the decomposition of water, that is to say, to the presence in the baths, of oxygen and 40 hydrogen due to the presence of free acid, it has been suggested to use sulfurous gas, chlorin, air deprived of its oxygen, etc. It has been even suggested to add to the baths oxidizing or reducing substances, according 45 to the result to be obtained, but always without appreciable success, all these at-

tempts having failed owing to the formation of hydrogen or oxygen or both gases, according to individual cases.

The present invention has for its object an electrolytic process for refining metals which process is exempt from the drawbacks hereinbefore mentioned, and which is suitable for obtaining all usual metals such as iron, copper, zinc aluminum, manganese, titanium, bromium, and the like.

The following are examples of the salts which may be used in carrying out this process:

|                                                                    |                                                                    |    |
|--------------------------------------------------------------------|--------------------------------------------------------------------|----|
| ZnSO <sub>4</sub> 7H <sub>2</sub> O                                | FeSO <sub>4</sub> 7H <sub>2</sub> O                                | 70 |
| CuSO <sub>4</sub> 5H <sub>2</sub> O                                | MnSO <sub>4</sub> 7H <sub>2</sub> O                                |    |
| NiSO <sub>4</sub> 7H <sub>2</sub> O                                | Ti(SO <sub>4</sub> ) <sub>2</sub> 3H <sub>2</sub> O                |    |
| Al <sub>2</sub> (SO <sub>4</sub> ) <sub>3</sub> 18H <sub>2</sub> O | Cr <sub>2</sub> (SO <sub>4</sub> ) <sub>3</sub> 7H <sub>2</sub> O. |    |

For metals having no sulfate, or if the sulfate of the metal is insoluble, another salt may be used, such for instance, as a chlorid.

In a crystallizable salt, such as for instance sulfate of zinc (ZnSO<sub>4</sub>7H<sub>2</sub>O) the water 7H<sub>2</sub>O contained in the crystal, forms an integral portion of the molecule ZnSO<sub>4</sub>H<sub>2</sub>O. It is therefore the water constituting the crystal or water of crystallization. It is not free, and the part played by it, cannot be compared to that of the water that would be used for dissolving this molecule, and called water of solution.

According to the present invention, the refining of a metal is produced by electrolyzing a bath containing a salt of this metal and not comprising any water but the water of crystallization of the salts forming the bath.

In order to prepare the electrolytic bath, a crystallized salt of the metal to be refined is subjected to the action of heat, in such a manner as this salt is melted in its water of crystallization, or it will be dissolved in an alkaline or earthlike sulfate, melted by means of heat in its water of crystallization.

For the purpose of liberating the baths of water of solution or "free water," in the first series of experiments water of crystallization of sulfate of magnesia MgSO<sub>4</sub>7H<sub>2</sub>O has previously been used for the purpose of dissolving the sulfate of the metal to be refined, and it has been found possible to dissolve in sulfates of magnesia, soda, potash, etc., dissolved in their water of crystallization, sulfates of iron, zinc, nickel, copper, etc. A bath thus constituted is an excellent one for

refining metals. This method may be replaced by a simpler one giving much better results: When any salt is dissolved in its water of crystallization, a portion or the 5 whole of this water evaporates, and the salt passes into the anhydrous state, or, if the temperature is too high, it becomes decomposed. If, however, during the dissolving of this salt in its water of crystallization, a 10 given quantity of water of solution is added for each salt in question, the bath always remains liquid and after the subsequent operation will contain, at the moment of its use, only the quantity of water corresponding to 15 that contained in the weight of the crystallized salt used. In fact, if the bath is allowed to cool, the salt will crystallize in a solid mass without mother liquor. A bath thus prepared, remains liquid provided that 20 its temperature is kept up at a slightly higher level than that at which it would become crystallized by cooling. It is thus possible to prepare the electrolytic bath by heating a salt of the metal considered containing 25 no water of dissolution. From time to time, a little water is added merely to compensate for the small quantity of water of crystallization which evaporates.

When an electrolytic operation is effected 30 with a bath prepared, the generation of oxygen and hydrogen is done away with, for in the bath in question, the water does not seem to be exposed to the decomposing action of the current. It appears to have for its function merely to keep up the constitution of the molecules of the molten salt, and the whole reaction takes place as if one had to deal with a fused salt.

During the refining operation, as soon as 40 the metal of the electrolyte is separated from the acid in order to settle on the cathode, the said acid becomes concentrated on the anode and attacks it, in order to reconstitute the electrolyte. Consequently, the 45 bath always retains its acid saturated with metal, that is to say, it always has the same richness or proportion of salt. The bath will therefore always remain not only concentrated, but saturated. Owing to that 50 fact, no decomposition of water takes place. Moreover, the water of this bath is always in combination, and never free. If it is de-

sired to refine according to the invention a piece of cast iron, this piece will be taken as anode and the electrolytic bath will be 55 obtained by melting in its water of crystallization the molecule  $\text{FeSO}_4 \cdot 7\text{H}_2\text{O}$ . During the electrolysis, the iron settles on the cathode, while the group  $\text{SO}_4$  in nascent state attacks the cast iron for producing  $\text{FeSO}_4$  60 which, with the  $7\text{H}_2\text{O}$ , reconstitutes the molecule  $\text{FeSO}_4 \cdot 7\text{H}_2\text{O}$  of the bath.

Having now particularly described and ascertained the nature of my said invention and in what manner the same is to be performed, I declare that what I claim is:—

1. An electrolytic process for refining metals consisting in placing an anode and a cathode in an electrolyte consisting of a salt of the metal to be refined but no water 70 except the water of crystallization of the salts in presence and passing a current from the anode through the electrolyte to the cathode.

2. An electrolytic process for refining 75 metals consisting in placing an anode and a cathode in an electrolyte consisting of a salt of the metal to be refined but no water except the water of crystallization of the salts in presence, the electrolytic bath being 80 prepared by melting a salt of the metal to be refined, and adding only the amount of water which is necessary for replacing the water of crystallization evaporated in the bath, owing to the heating and passing an 85 electric current through the anode, electrolyte and cathode.

3. An electrolytic process for refining metals consisting in placing an anode and cathode in a bath containing a salt of the 90 metal to be refined but no water except the water of crystallization of the salts in presence, the electrolytic bath being prepared by solving a salt of the metal to be refined in an alkaline or earthlike sulfate 95 melted by means of heat in its water crystallization and passing a current through said anode, bath and cathode.

In testimony whereof I affix my signature in presence of two witnesses.

NICOLAS HENRI MARIE DEKKER.

Witnesses:

H. C. COXE,  
J. BEE.